

# UNITED STATES PATENT OFFICE.

FRANK P. VAN DEN BERGH, OF BUFFALO, NEW YORK.

## PROCESS OF MANUFACTURING ALKALI SILICATES.

SPECIFICATION forming part of Letters Patent No. 677,906, dated July 9, 1901.

Application filed August 3, 1900. Serial No. 25,821. (No specimens.)

To all whom it may concern:

Be it known that I, FRANK P. VAN DEN BERGH, a citizen of the United States, residing at Buffalo, in the State of New York, have 5 invented certain new and useful Improvements in Processes of Manufacturing Alkali-Metal Silicates; and I do hereby declare the following to be a full, clear, and exact description of the invention, such as will enable 10 those skilled in the art to which it appertains to employ the same.

More particularly, my invention relates to a new and improved art or process for the production of alkali-metal silicates from sodium chlorid or potassium chlorid or other materials containing sodium or potassium or 15 their salts and a silicious substance or substances by means of heat and electrolysis, one or both being produced by an electric 20 current in the presence of an oxidizing agent or agents.

In carrying out my invention I use sodium chlorid or potassium chlorid or others suitable materials containing sodium or potassium or 25 their salts and a suitable silicious substance—such as silica, sand, silex, quartz, cullet, feldspar, or other suitable material—and these are reduced to a molten mass within the furnace-chamber by the heat of the 30 electric current, either with or without the auxiliary heat of internal or external combustion. This fusion of the materials is caused to take place in an atmosphere which contains an excess of oxygen, which is supplied by any suitable means—such as iron 35 oxid, manganese oxid, the sulfate, nitrate, or other oxygen-yielding salt of sodium or potassium, or other suitable solid which may be mixed with the materials fed into the fur-

40 nace, or by water, steam, air, oxygen, ozone, or other suitable oxygen-yielding liquid or gas which may be injected into the furnace, so that the decompositions and reactions which take place in the molten bath or with- 45 in the furnace-chamber and the products resulting therefrom take place and are in the presence of an excessive supply of free oxygen or oxygen which is in the nascent state. The principal purpose of such oxidation is to avert 50 the formation of sodium or potassium silicid or of certain silicates of incomplete oxidation—that is, containing a less relative pro-

portion of oxygen—and to insure the formation of the normal or ortho silicates of sodium or potassium. This bath or molten mass is 55 subject to intense heat and to electrolysis, one or both due to the electric current, the heat principally serving to reduce the materials to a fluid condition and the electrolysis serving principally to effect decomposition of 60 the materials.

The sodium or potassium salts and the silicious material being together introduced into the furnace, the first effect is to fuse these materials. Subsequently the salts under 65 the influence of the electric current are decomposed, and the resulting gas or gases, as chlorin, in the case of sodium or potassium chlorid, are liberated and conducted away through a suitable conduit leading from the 70 furnace and utilized by any of the methods in use for the manufacture of hydrochloric acid, liquid chlorin, bleaching-powder, hypochlorite solutions, or other products of value in the arts. 75

The principal reaction which takes place and that which is essential to carrying out my process may be expressed by the following empirical formula:



In preparing the mixture to be fed into the furnace the composition of the materials is to be observed with care, and they are to be added in such proportions and with such admixtures of auxiliary electrolytes or fluxes 90 as to secure and maintain fusion at the lowest temperature and to secure and maintain decomposition by electrolysis with the greatest economy as to materials, time, and current. For instance, when operating with sodium chlorid a small proportion of a potassium salt will result in a lowering of the fusing-point of the bath and will at the same time facilitate electrolysis. 95

It is desirable that the resulting silicate 100 should be as fluid as possible, as well after it issues from the furnace as when molten therein, and to this end care must be exercised as to the proportions of the materials used.

Thus from two to four times as much of the sodium chlorid as of the silicious material should be used, for if a much greater proportion of silica is employed there is a liability 5 of hard silicates being formed instead of the liquid silicate or "water-glass."

In operating according to my process the "rock salt" or other material containing the alkali-metal base and the silicious material 10 are first broken or crushed to such a condition as to permit and facilitate feeding them into an electric furnace and also to facilitate their fusion. The electric furnace employed may be of any desired type, provided it has 15 a properly-closed chamber and a proper exit for the vapors generated connected with a condensing apparatus. It is especially advantageous, however, to employ a furnace affording a continuous process of reduction— 20 that is, of fusion and decomposition—and a furnace well adapted for this purpose has heretofore been designed by me and upon which Letters Patent were issued to me under date of July 4, 1899, and bearing number 25 626,373.

The material to be treated is introduced into the furnace and brought into contact with the electric current and is rapidly converted into a molten mass. The exact amount of 30 silicious material which is used cannot be stated arbitrarily owing to the variations in the character and richness of the materials which may be used and must be in each case relatively determined, as it may be by any 35 person skilled in the art of smelting ores. Likewise the volume and quantity of the electric current employed, as hereinbefore set forth, for the purposes of heat and electrolysis will be determined by the work being done 40 and the character of the materials being treated.

For the complete and certain oxidation and hydration of the molten mass it is usually desirable to project a jet of steam or air directly 45 into the furnace, and its quantity must also be determined by the quality of the native materials being operated upon and their quantity. However, the material used in carrying out my process is such and its physical condition, being broken into small pieces, is such 50 that large volumes of air are necessarily delivered into the furnace-chamber along with the material. The materials used also carry with them a considerable and often very large 55 amounts of water, so that it is not always necessary to introduce the steam into the furnace. Whether or not this is necessary has to be determined by the condition of the materials being operated upon.

60 The molten silicate or mixture of silicates in the condition of "soluble glass" is caused to flow away from the furnace into a proper receptacle, vat, or tank containing water, wherein it may be further treated in such 65 manner as may be desired—as, for instance, by the passage of carbon dioxid through the

liquid, thus decomposing the fluid silicate with the formation of carbonate of sodium and the liberation of silica as hydrated silica, or by the addition of "milk of lime" causing 70 the decomposition of the alkali-metal silicate with the formation of silicate of calcium and the liberation of the alkali as caustic soda or caustic potash. I do not, however, restrict or limit my invention to the particular means 75 described for carrying out the process, as any one and all of them may be varied without departing from the spirit of my invention, and I do not limit myself to the use of steam or water-vapor as an oxidizing agent, as oxygen or air, ozone, hematite iron ore, or other suitable material capable of yielding a large proportion of oxygen when subjected to the heat and energy of the electric current within the furnace may be employed, and these oxygen-yielding materials may be heated separately from the sodium or potassium yielding materials, as is sometimes desirable. 80 85

Having thus described my invention, what I claim, and desire to secure by Letters Patent, is—

1. The herein-described process of manufacturing alkali-metal silicates, which consists in subjecting a substance containing an alkali-metal base, and a silicious substance in 95 the presence of oxygen, to heat and electrolysis, to fuse the mass and drive off the acidulous elements or oxids, and combine the base and silica to form an alkali-metal silicate, substantially as set forth. 100

2. The herein-described process, of manufacturing alkali-metal silicates, which consists in subjecting an alkali-metal chlorid and a silicious substance to heat sufficient to fuse the same, and to electrolysis to drive off the 105 chlorin and permit the combination of the alkali-metal base with the fused silica in the presence of oxygen, substantially as set forth.

3. The herein-described process of manufacturing alkali-metal silicates, which consists in subjecting an alkali-metal chlorid and a silicious substance, in the proportion of approximately three parts of chlorid to one of the silicious substance, to heat and electrolysis in the presence of oxygen, substantially 110 115 as set forth.

4. The herein-described process of manufacturing alkali-metal silicates, which consists in subjecting sodium chlorid and a smaller proportion of potassium chlorid, and a substance containing silica, to heat and electrolysis in the presence of oxygen, the potassium chlorid serving to lower the fusing-point of the bath, and also to facilitate the electrolysis, substantially as set forth. 120 125

5. The herein-described process of manufacturing alkali-metal silicates containing a high proportion of oxygen, which consists in subjecting a substance containing an alkali-metal base, and a silicious substance to heat 130 and to electrolysis, ample to fuse the materials and drive off the acidulous constituents, 135

such operations taking place in an atmosphere containing an excess of oxygen, substantially as set forth.

6. The herein-described process of manufacturing orthosilicate of sodium, which consists in subjecting sodium chlorid and silica to heat and electrolysis in the presence of oxygen, whereby these are fused and the following expressed reaction takes place:



7. The herein-described process which consists in subjecting to heat and electrolysis in the presence of oxygen an alkali-metal chlorid, and a silicious substance to form an alkali-metal silicate, and then treating the silicate so formed to produce a caustic alkali, substantially as set forth. 15

FRANK P. VAN DENBERGH.

Witnesses:

GEO. J. MAY, Jr.,  
LEWIS I. O'NEAL.